

## UNITED STATES PATENT OFFICE.

HARRY GREGG GRINLINTON, OF NORTH SYDNEY, NEW SOUTH WALES, AUSTRALIA.

## COATING OF METALS WITH METALS OF A LOWER FUSING POINT.

No Drawing.

Application filed June 14, 1920. Serial No. 366,923.

*To all whom it may concern:*

Be it known that I, HARRY GREGG GRINLINTON, a subject of the King of Great Britain, residing at North Sydney, in the State 5 of New South Wales, Commonwealth of Australia, have invented certain new and useful Improvements in the Coating of Metals with Metals of a Lower Fusing Point, of which the following is a specification.

10 This invention relates to improvements in the coating of metals and their alloys with metals or alloys of a lower fusing point, but exclusive of aluminium and its alloys, and has especial reference to the coating of metals 15 in sheet form.

Heretofore the methods in use for coating metals and their alloys have not been always commercially successful inasmuch as there has been a great waste of metal and material 20 in addition to which, considerable labor has been expended in removing the oxides from or otherwise cleaning the metal preparatory to applying the compound containing the coating metal.

25 The present invention consists in the process of applying the compound containing the coating metal.

In carrying out the process the surface of the foundation metal to be coated is preferably 30 first rubbed with emery paper or the like or other known mechanical means employed to remove any foreign matter but dispensing with the use of sulphuric and like acids or cyanides. The surface has then 35 applied to it with a brush or the like a dressing of the coating compound which should be first well agitated, care being taken that it is evenly distributed.

A flux, consisting of powdered stearic acid, 40 is then sprinkled over the whole area and dressed and the metal passed slowly over suitable heating apparatus. This preferably is a Bunsen burner of sufficient length to heat simultaneously the width of the metal 45 sheet or object.

When the coating metal becomes totally fused, say between 232° C. and 288° C., in the case of tin, but not at so high a temperature as to cause the stearic acid or other flux to be completely volatilized and while the 50 foundation metal is still hot and the coating metal fluid, the surface is wiped with a cloth or pad leaving the coating metal in close union with the foundation metal.

The coating compound consists of a proportion of the coating metal in very fine particles, ammonium or other like volatilizable chloride together with a medium such as glycerine and a small proportion of water and preferably a volatilizable metal chloride. 55

As an example, in coating a metal such as copper or brass with tin, I employ a tinning compound consisting of,

Tin in very fine particles approximately 10 parts, ammonium chloride approximately 65 20 parts, glycerine approximately 15 parts, aqua approximately 10 parts, to which I may add, zinc chloride approximately 45 parts.

The very fine particles of the coating metal are preferably obtained by atomization such as by injecting a strong current of air against a jet of the molten metal. 70

Having thus described my invention, what I claim as new and desire to protect by Letters Patent is:—

In the coating of metals such as copper or brass or their alloys with tin, applying a dressing of tin in a fine state of division with a suitable medium to the foundation metal, sprinkling powdered stearic acid as a flux 80 over the area dressed, applying heat until the coating metal is totally fused but prior to the complete volatilization of the flux and then wiping the fluid coating metal with a cloth or pad substantially as described. 85

In testimony whereof I have hereunto set my hand,

HARRY GREGG GRINLINTON.